

# UNITED STATES PATENT OFFICE.

JOHN BILBIE AND HENRI DRIVET, OF LONDON, ENGLAND.

## PROCESS OF TREATING CARBID OF CALCIUM.

SPECIFICATION forming part of Letters Patent No. 650,747, dated May 29, 1900.

Application filed October 6, 1898. Serial No. 692,827. (No specimens.)

*To all whom it may concern:*

Be it known that we, JOHN BILBIE, a subject of the Queen of Great Britain, and HENRI DRIVET, a citizen of the Republic of France, both residing in the city of London, England, have invented a certain new and useful Process of Treating Carbide of Calcium, (for which application has been made in Great Britain, No. 19,786, dated September 17, 1898,) of which the following is a specification.

The objects attained by our invention are to render the commercial carbide of calcium proof against the action of atmospheric moisture, to neutralize or destroy its objectionable odor, to render the production of gas in the presence of water more uniform, and to enrich the gas and improve its lighting power.

By treating carbide of calcium in a broken or granulated condition with a small percentage of petroleum in such a manner as to coat the pieces or grains of carbide with a thin film of the oil the carbide will be rendered practically weatherproof, and when used in generators or lamps it will combine with water in such a manner as to produce the gas regularly and prevent the excessive and oftentimes violent evolution of gas, which is often experienced in using the ordinary carbide. Moreover, the oil is taken up by the gas produced, with the effect of improving its quality and increasing its lighting power.

For the purpose of coating the carbide we prefer to use petroleum previously purified by quicklime. The petroleum is applied by sprinkling it on the granulated carbide and stirring the mass until the grains are thor-

oughly and uniformly coated with the oil. From two to five parts of petroleum will suffice for one hundred parts of carbide.

To kill the natural odor of the carbide and impart to it a pleasant odor, we treat the carbide with essential oil—such as citronella, mirbane, or eucalyptus. We preferably treat the carbide with from two to five per cent. of essential oil before the treatment with petroleum and give it a second treatment with the essential oil after the treatment with petroleum, the carbide being stirred after each treatment to thoroughly incorporate the essential oil with it.

The above treatment preserves the carbide, renders it agreeable to handle, enriches the gas, and renders the production of gas in lamps and generators steady and uniform.

Having described our invention, what we claim is—

The improved process of treating carbide of calcium consisting in treating the pieces or grains thereof with an essential oil, then coating the pieces or grains with petroleum, and finally again treating the carbide with an essential oil, substantially as described and for the purpose set forth.

In testimony whereof we have hereunto set our hands in the presence of the two subscribing witnesses.

JOHN BILBIE.  
HENRI DRIVET.

Witnesses:

ALFRED NUTTING,  
FRED. G. LUNNON.